

## UNITED STATES PATENT OFFICE

2,447,539

## TREATMENT OF WOOL

John B. Rust, Montclair, N. J., assignor to Montclair Research Corporation, a corporation of New Jersey

No Drawing. Application November 16, 1944,  
Serial No. 563,791

6 Claims. (Cl. 260—29.7)

1

This invention relates to fiber treatment and particularly to processes of treating wool to reduce substantially the shrinkage of wool, to products obtained by such processes of treatment and to baths utilized in such treatment.

It is known that it is possible to produce non-felting and non-shrinking wool by chlorination or bromination of wool. There have also been described processes of producing non-felting wool by treatment with alcohol solutions of alkalis, by treatment with sulfuryl chloride, nitrosyl chloride, and the like. (However, in this case mixed cotton and woolen goods cannot be treated.)

Treatment with rubber latex in the presence of quaternary ammonium, phosphonium, sulfonium compounds and the application of alkylated methylol melamine in relatively high temperatures have also been described.

In the prior art processes difficulties are encountered, including danger of damage to fibers, reducing wearing qualities and undesirable hand, which are hard to prevent in most of the former processes.

Processes have also been suggested for the use of synthetic resins, such as methacrylate resins, butadiene polymers, etc., for the treatment of a wide variety of fibers. Those suggestions in the art treat all of these polymeric substances as equivalent for all fibers. But investigation proves that such suggestions are erroneous because while such resins and polymers can be applied to wool for example, they are not equally efficacious in effecting a shrink-proofing effect. Effective shrink-proofing requires definite conditions and compositions and the determination of such conditions and compositions is a matter that cannot be predicted with reasonable certainty.

In prior application Serial No. 537,537, filed May 26, 1944, entitled Woolen treatment and products therefor, in the name of John B. Rust, it has been disclosed that no shrink-proofing effect whatever is obtained unless a straight butadiene polymer is used or some polymer in which butadiene is present to a major extent. The present invention is a continuation of the work leading to effect shrink-proofing of fibers specifically wool.

Among the objects of the present invention is a treatment of wool and wool containing fabrics to render them substantially resistant to felting.

2

fulling and shrinkage by relatively simple processes and particularly where the danger of damage to fibers, reducing wearing qualities and undesirable hand are eliminated.

5 Other objects include the production of treating baths enabling the conditioning of wool to produce products of the character set forth above.

Other and further objects and advantages of the present invention will appear from the more detailed description set forth below, it being understood that this more detailed description is given by way of illustration and explanation only and not by way of limitation since various changes therein may be made by those skilled in the art without departing from the scope and spirit of the present invention.

In accordance with the present process the wool either as raw wool, yarn, knit, woven goods or mixed goods is entered into an aqueous conditioning bath containing an interpolymeric butadiene derivative from butadiene and a methacrylic derivative, specifically an ester, having the general formula



where R is some aryl or alkyl radical having less than 8 carbon atoms such as methyl, ethyl, propyl, butyl, amyl, benzyl and the like, and exhausting the bath on the fiber. The bath desirably should contain the butadiene interpolymer in an amount to give, under the conditions of treatment, a wool having from 1% to 25% of interpolymer based on the weight of the wool.

35 The bath is conditioned by adding to it a sufficiently strong electrolyte to allow the deposition of the interpolymeric butadiene derivative on the wool fibers. It has been found that in such a bath no deposition of the interpolymeric butadiene derivative occurs under ordinary conditions.

40 However, upon addition of an electrolyte, exhaustion of the bath will take place with varying rapidity, depending mainly upon temperature and electrolyte concentration. Without any limitation by way of theoretical considerations, it is believed that reversal of the electrical charge on the colloidal particles of the interpolymeric butadiene derivative takes place on addition of the electrolyte enhancing the affinity of the interpolymeric butadiene derivative for the fiber. The

45

proportion of electrolyte added would be insufficient to account on a theoretical basis for the salting out of the interpolymeric butadiene particles. Thus the effect must be one of electrical charge rather than precipitation by coagulation. When the electrolyte is added to the treated bath there is no coagulation or precipitation even on heating for long periods of time. It is only in the presence of the wool that deposition occurs. This is additional proof that electrical charge of the particles is involved rather than a salting effect.

It has furthermore been found that as the methacrylic ester content of the interpolymeric butadiene derivative of this invention is increased, shrinkage proofing of the wool decreases rapidly, beyond certain limits. Thus an emulsion of about 6% of interpolymeric butadiene derivative containing 80% of methacrylic ester will deposit readily on the wool but no shrinkage proofing is obtained in this manner. However, if the methacrylic ester content of the interpolymeric butadiene derivative is decreased to 10% excellent shrinkage proofing is obtained from the treated wool. This effect is both startling and noteworthy since it appears that the shrinkage proofing effect is directly proportional to the butadiene concentration in the interpolymeric. Thus it has been found that up to about 20% of methacrylic ester may be used in the interpolymeric without any deleterious effect upon the shrinkage proofing efficiency of the emulsion. In fact the proportion of methacrylic ester within the acceptable range appears to have some beneficial effect inasmuch as for example, in some cases increased abrasion resistance is obtained in the treated wool.

Consequently the methacrylate derivative is utilized with the butadiene in producing the interpolymer, so that the amount of methacrylate derivative present, is insufficient to interfere with the desired shrink-proofing effect desired while at the same time the amount of methacrylate derivative is sufficient to give some special effect on properties in the treated wool which would not be obtainable in its absence.

In the prior art it has been proposed to deposit various synthetic resins and plastics from emulsions onto textile materials. There has been no hint that by varying the composition of such resin emulsions a variation in the physical properties of the treated textile can be obtained.

It has been found that the acceptable range of methacrylate component in the butadiene interpolymers varies with the type of methacrylate derivative. Thus in the case of the present invention where a methacrylic ester is used the acceptable maximum limit of methacrylic ester as stated above is 20% in the butadiene interpolymer, however as high as 50% of the methacrylic ester may be used with definite shrink-proofing occurring. Higher than 50%, however, appears to be inoperative. As with other derivatives, this limit is not the same.

The electrolyte content may vary over substantial limits but sufficient electrolyte should be present to condition the bath so that the bath, although stable in the presence of wool fibers, will deposit the polymer in the presence of the conditioning electrolyte. Thus the electrolyte content may vary from about 25% to about 500% based on the weight of the interpolymeric butadiene derivative present. The following are exemplary: sodium sulfate, sodium chloride, sodium bromide, sodium iodide, sodium sulfite, sodium bisulfate, sodium bisulfite, sodium nitrate,

sodium acetate, and the like, or salts of the above used potassium, lithium, caesium and so forth in place of sodium. Salts like zinc chloride may also be used where the coagulation does not appear to be too serious since it occurs in small particulate form and the particles may be redispersed by stirring. As such electrolyte, water-soluble salts may be used, desirably such salts which do not precipitate the polymer, neutral

10 salts, specifically salts of strong bases and strong acids, particularly inorganic salts, are preferred. The term "conditioning electrolyte" is used hereinafter to cover such electrolytes which produce the desired deposition of the polymer. It has been found that it is possible to deposit the emulsions of the present invention on wool at pH of seven or even slightly higher. However, it is preferred to operate at a pH of seven or below since under these latter conditions more rapid dispersal is effected.

20 The operation is desirably carried out at a temperature sufficient to give exhaustion of the bath with the particular emulsion being used. This will vary with different emulsions. While

25 lower temperatures may be used, the operation is desirably carried out at temperature ranges from 40° C. to the boiling point of the bath. The polymer can be applied before or after fulling, weaving, scouring and the like operations. In

30 some cases it can be applied in the dye bath. Mixed goods including wool-cotton, wool-rayon and so forth can be treated by this method without any deleterious effect. If desired the wool may be subjected to a pretreatment, as for example, chlorination or bromination, before being

35 treated in accordance with the present invention. In emulsions containing the methacrylate-butadiene interpolymer the emulsifying agent may be any anionic emulsifying agent which is

40 stable at or below pH7. Such emulsifying agents are exemplified by sodium auryl sulfonate, sodium alkyl naphthalene sulfonates, long chain alkyl sodium sulfonates or sulfates, sodium dioctyl sulfosuccinate and so forth. There may also be used neutral non-cationic emulsifying agents such as mannityl monolaurate, the reaction products of protein derivative products with acid chlorides, ethylene oxide reaction products with fatty acids, fatty alcohols and the like.

45 50 Emulsions of the interpolymers used in accordance with the present invention are preferably but not necessarily those which have been carried to a 100% polymerization. When 100% polymer is obtained, considerable cross linking

55 occurs in the polymer with consequent insolubility in organic solvents. Thus a type of pre-vulcanizing of the polymer has been obtained. It is also possible to vulcanize the interpolymers with mixtures of vulcanizing accelerators such as thiuram

60 disulfide and so forth, vulcanizing agents such as sulfur, dinitrobenzene, alkyl phenol sulfide and so forth, either previously or subsequently to deposition or dyeing into the wool fibers.

65 The treatment of wool fibers is particularly emphasized herein, although animal fibers such as silk and protein fibers such as "Aralac" (a casein fiber) may also be treated in accordance with this invention.

70 After treatment in accordance with the present invention, the wool is rinsed and dried. Its properties have been altered to such a degree that it no longer has a tendency to felt during washing and consequently is non-shrinking. Although it is not intended that the invention be limited by theoretical considerations, it is thought that the

interpolymeric particles applied as set forth in this description distribute themselves among the fibers of the wool and in some instances fill the interstices of the wool scales, thus preventing an intertwining and consequent felting of the wool. Thus the deposited interpolymer would prevent intertwining of the wool fibers and also permit relatively easy slippage of the fibers one on the other.

Exemplifying the present invention the following examples are given:

*Example 1.*—A series of butadiene-methyl methacrylate emulsions was prepared using butadiene and methyl methacrylate in the proportions shown in columns A and B of Table I.

Table I

|   | A<br>Parts<br>Butadiene | B<br>Parts<br>Methyl<br>Methacry-<br>late |
|---|-------------------------|-------------------------------------------|
| 1 | 45                      | 5                                         |
| 2 | 40                      | 10                                        |
| 3 | 35                      | 15                                        |
| 4 | 30                      | 20                                        |
| 5 | 25                      | 25                                        |
| 6 | 20                      | 30                                        |
| 7 | 15                      | 35                                        |
| 8 | 10                      | 40                                        |

In all cases the butadiene was condensed in pressure reactors cooled to below  $-5^{\circ}\text{ C}$ . While the reactors were kept in the freezing mixture the methyl methacrylate, which had previously been distilled, was added, followed in each case by 100 parts of a buffer solution of pH 11, 5 parts of 30% hydrogen peroxide and 5 parts of sodium lauryl sulfate. The buffer solution consisted of 358 parts of disodium phosphate and 7.16 parts of trisodium phosphate dissolved in 980 parts of distilled water. The reactors were then taken out of the freezing mixture and closed immediately.

The reactors were left standing for about 2 hours and allowed to come to room temperature. They were then heated under controlled conditions to  $45^{\circ}\text{ C}$ . and agitated continuously. The reactors were taken out of the bath after 24 hours, cooled and opened. None of the reactors showed any pressure on opening. Complete polymerization was thus indicated and the solid content of each of these emulsions was 33 1/3%.

*Example 2.*—The emulsions made according to Example 1 were applied to hand knit sample of wool approximately 7" x 5" in size. For each wool sample an amount of emulsion of Example 1 containing a weight of solids corresponding to 6% of the weight of the wool sample was weighed out. The emulsions were added to 200 parts of water, and the bath was conditioned with anhydrous sodium sulfate. Then 10% sulfuric acid was added to bring the pH of the bath to below 7. The wool samples which weighed approximately 15 parts were then immersed in the cold bath and agitated continuously. After one hour at room temperature the bath had not yet cleared up. The bath was, therefore, heated to boiling. After 15 minutes the bath was exhausted. The wool samples were taken out of the bath, rinsed with warm water and dried.

The wool samples were then washed in a washing machine for 3 hours using a 1/4% soap solution at  $80^{\circ}\text{ C}$ . The samples were then rinsed and dried. The extent of the felting and shrinking caused by the washing is shown in column C of Table II.

Table II

|   | A<br>Parts<br>Butadiene | B<br>Parts<br>Methyl<br>Methacry-<br>late | C<br>Felting and<br>Shrinking |
|---|-------------------------|-------------------------------------------|-------------------------------|
| 1 | 45                      | 5                                         | Slight.                       |
| 2 | 40                      | 10                                        | Considerable.                 |
| 3 | 35                      | 15                                        | Bad.                          |
| 4 | 30                      | 20                                        | Do.                           |
| 5 | 25                      | 25                                        | Do.                           |
| 6 | 20                      | 30                                        | Do.                           |
| 7 | 15                      | 35                                        | Do.                           |
| 8 | 10                      | 40                                        | Do.                           |

15 The sample containing 10% methyl methacrylate stood up well in the washing, while the sample with 20% methyl methacrylate showed a noticeable improvement over untreated wool. The felting increased with the percentage of 20 methyl methacrylate in the sample.

*Example 3.*—A series of ethyl methacrylate-butadiene emulsions was made up. The two monomers were used in the proportions indicated in 25 columns A and B in Table III.

Table III

|   | A<br>Parts<br>Butadiene | B<br>Parts Ethyl<br>Methacry-<br>late |
|---|-------------------------|---------------------------------------|
| 1 | 45                      | 5                                     |
| 2 | 40                      | 10                                    |
| 3 | 35                      | 15                                    |
| 4 | 30                      | 20                                    |
| 5 | 25                      | 25                                    |
| 6 | 20                      | 30                                    |
| 7 | 15                      | 35                                    |
| 8 | 10                      | 40                                    |

30 The butadiene was passed over calcium chloride and condensed in pressure reactors which were cooled to below  $-5^{\circ}\text{ C}$ . The pressure reactors were then emptied into a Dewar flask, and the butadiene kept in there until added to the reaction mixture.

45 The ethyl methacrylate, which had been distilled previously, was poured into the pressure reactors. In all cases 100 parts of buffer, 5 parts of 30% hydrogen peroxide solution and 5 parts of sodium lauryl sulfate were added, while the pressure reactors were still kept in the 50 freezing mixture. The buffer solution had been made up from 35.8 parts of disodium phosphate and 7.16 parts of trisodium phosphate dissolved in 980 parts of water. The butadiene was added 55 last to the reaction mixture in the pressure reactors and the reactors were closed. The reactors were allowed to come to room temperature and were then put in an agitator with a constant temperature bath at  $45^{\circ}\text{ C}$ .

60 Except for emulsion #1, all reactors were taken out after 21 hours in the agitator. The reactor with emulsion #1 was taken out after 27 hours. The reactors were cooled and opened. The reactor with emulsion #1 showed a very slight pressure, but no foaming on opening. None of the 65 other reactors showed any pressure or foaming. This indicated complete polymerization in all cases, and the solid content of each of these emulsions was therefore, 33 1/3%.

70 *Example 4.*—The emulsions made according to Example 3 were applied to hand knit wool samples approximately 7" x 5" in size. An amount of emulsion containing solids corresponding to 6% of the weight of the wool sample to be 75 treated was weighed out and added to 200 parts

of water. The weights of the wool samples and the corresponding amounts of emulsion are given in columns C and D of Table IV. The bath was conditioned in each case with an electrolyte consisting of 1.0 part of anhydrous sodium sulfate, and 1.0 part of 10% sulfuric acid was added. The wool sample was immersed in the cold bath, and the bath then heated to 60-70° C. After 20 minutes at this temperature the bath had not yet cleared up, and another portion of 1.0 part of anhydrous sodium sulfate was added to each bath. Emulsions #1 and #2 cleared up completely after 60 minutes at 60-70° C., thus indicating complete exhaustion in the bath. The other emulsions still showed a haze even after 80 minutes at 60-70° C., and the haze, which increased from emulsion #3 to #8, did not seem to disappear. The samples were taken out of the bath, rinsed and dried.

Table IV

|   | A<br>Parts<br>Butadiene | B<br>Parts<br>Ethyl<br>Methacrylate | C<br>Parts<br>Wool | D<br>Parts<br>Emulsion | E<br>Felting and<br>Shrinking |
|---|-------------------------|-------------------------------------|--------------------|------------------------|-------------------------------|
| 1 | 45                      | 5                                   | 14.70              | 2.64                   | Fair.                         |
| 2 | 40                      | 10                                  | 15.95              | 2.87                   | Do.                           |
| 3 | 35                      | 15                                  | 14.60              | 2.64                   | Considerable.                 |
| 4 | 30                      | 20                                  | 14.95              | 2.69                   | Do.                           |
| 5 | 25                      | 25                                  | 14.78              | 2.66                   | Do.                           |
| 6 | 20                      | 30                                  | 14.78              | 2.66                   | Bad.                          |
| 7 | 15                      | 35                                  | 15.95              | 2.87                   | Do.                           |
| 8 | 10                      | 40                                  | 14.53              | 2.62                   | Do.                           |

All eight wool samples were given 6 washings of one hour each in a washing machine containing a 1/2% soap solution at 70° C. They were then rinsed and dried.

The extent of the felting and shrinking caused by the washings is shown in column E of Table IV. The lower percentages of ethyl methacrylate stand up better than the higher percentages and up to 50% ethyl methacrylate a definite improvement over untreated wool can be noticed. Even the 60% ethyl methacrylate sample showed a slight improvement over untreated wool.

*Example 5.*—A series of butadiene-butyl methacrylate emulsions was prepared, using butadiene and butyl methacrylate in the proportions shown in columns A and B of Table V.

Table V

|   | A<br>Parts<br>Butadiene | B<br>Parts Butyl<br>Methacry-<br>late |
|---|-------------------------|---------------------------------------|
| 1 | 45                      | 5                                     |
| 2 | 40                      | 10                                    |
| 3 | 35                      | 15                                    |
| 4 | 30                      | 20                                    |
| 5 | 25                      | 25                                    |
| 6 | 20                      | 30                                    |
| 7 | 15                      | 35                                    |
| 8 | 10                      | 40                                    |

In all cases the butadiene, which had been passed over calcium chloride, was condensed in pressure reactors cooled to below -5° C. While the reactors were kept in the freezing mixture the butyl methacrylate, which had previously been distilled, was added, followed in each case by 100 parts of a buffer solution of pH 11, 5 parts of 30% hydrogen peroxide and 5 parts of sodium lauryl sulfate. The buffer solution consisted of 35.8 parts of disodium phosphate and 7.16 parts

of trisodium phosphate dissolved in 980 parts of distilled water. The reactors were then taken out of the freezing mixture and closed immediately. The reactors were left standing for about 2 hours and allowed to come to room temperature. They were then heated under controlled conditions to 45° C. and agitated continuously. The reactors were taken out after 22 hours, cooled and opened. None of the reactors showed any pressure on opening. Complete polymerization was thus indicated and the solid content of each of these emulsions was 33 1/2%.

*Example 6.*—The emulsions made according to Example 5 were applied to hand knit samples of wool approximately 7" x 5" in size. For each wool sample an amount of emulsion of Example 1 containing a weight of solids corresponding to 6% of the weight of the wool sample to be treated was weighed out. Columns C and D in Table VI show the weights of the wool samples and the respective amounts of emulsion used. The emulsions were added to 200 parts of water and the bath was conditioned with an electrolyte consisting of 1 part of anhydrous sodium sulfate. Then 1 part of 10% sulfuric acid was added to bring the pH of the bath below 7. The wool samples were immersed in the wool bath, which was then heated to 60-70° C. and kept at that temperature. The wool sample was agitated in the bath continuously. After 20 minutes of 60-70° C. the bath was not yet exhausted and another portion of 1 part of anhydrous sodium sulfate was added. An hour later the bath was clear except for a slight haze, i. e. all the latex had been exhausted. The wool samples were taken out of the bath, rinsed with warm water and dried.

Table VI

|    | A<br>Parts<br>Butadiene | B<br>Parts<br>Butyl<br>Methacry-<br>late | C<br>Parts<br>Wool | D<br>Parts<br>Emulsion | E<br>Felting and<br>Shrinking |
|----|-------------------------|------------------------------------------|--------------------|------------------------|-------------------------------|
| 45 | 45                      | 5                                        | 13.00              | 2.34                   | Slight.                       |
| 2  | 40                      | 10                                       | 14.29              | 2.57                   | Do.                           |
| 3  | 35                      | 15                                       | 15.27              | 2.75                   | Do.                           |
| 4  | 30                      | 20                                       | 14.28              | 2.57                   | Considerable.                 |
| 5  | 25                      | 25                                       | 13.84              | 2.49                   | Bad.                          |
| 6  | 20                      | 30                                       | 12.58              | 2.28                   | Do.                           |
| 7  | 15                      | 35                                       | 14.58              | 2.62                   | Do.                           |
| 8  | 10                      | 40                                       | 17.20              | 3.10                   | Do.                           |

The wool samples were then washed in a washing machine using 25 parts of powdered soap for 13,000 parts of hot water at 70° C. The samples were given 6 washings of one hour each, and were rinsed and dried between washings. The extent of the felting and shrinking caused by the washings is shown in column E of Table VI. The lower percentages of butyl methacrylate stood up better. Best results were obtained with 30% butyl methacrylate or less, but even with 40% butyl methacrylate a definite improvement over untreated wool was noticeable.

Having thus set forth my invention, I claim:

1. The method of treating wool which comprises heating the wool in a bath of an aqueous emulsion at a temperature of from 40° C. to the boiling point of the bath containing a synthetic copolymer of 100% polymerization of butadiene-1,3 and from 5 to 50% based on the weight of the copolymer of a methacrylate ester, the esterifying group having less than 8 carbon atoms, and a non-cationic emulsifying agent in the presence of at least 25% by weight on the copoly-

mer of a water-soluble neutral salt of an alkali metal as conditioning electrolyte, the pH of the bath being below 7 to give deposition of from 1 to 25% by weight of polymer on the wool, the bath being substantially stable in the absence of the wool, the amount of the butadiene polymer being sufficient to give substantial shrinkproofing properties to the wool while retaining substantially its normal hand.

2. A bath for treating wool to give shrink-proofing with substantially normal hand which comprises an aqueous substantially stable emulsion containing a synthetic copolymer of 100% polymerization of butadiene-1,3 and from 5 to 50% based on the weight of the copolymer of a methacrylate ester, the esterifying group having less than 8 carbon atoms, in amount to give 1 to 25% by weight of polymer deposition on the wool, a non-cationic emulsifying agent, and at least 25% by weight on the copolymer of a water-soluble neutral salt of an alkali metal as conditioning electrolyte, the pH of the bath being below 7.

3. A bath as set forth in claim 2, in which the emulsifying agent is an anionic emulsifying agent.

4. A bath as set forth in claim 2, in which the ester is methyl methacrylate in an amount of not more than 20% based on the weight of the copolymer.
5. A bath as set forth in claim 2, in which the ester is ethyl methacrylate.
6. A bath as set forth in claim 2, in which the ester is butyl methacrylate in an amount of not more than 40% based on the weight of the co-polymer.

JOHN B. RUST.

#### REFERENCES CITED

The following references are of record in the 15 file of this patent:

#### UNITED STATES PATENTS

| Number       | Name          | Date          |
|--------------|---------------|---------------|
| 2,232,515    | Arnold et al. | Feb. 18, 1941 |
| 20 2,340,358 | Young         | Feb. 1, 1941  |
| 2,343,095    | Smith         | Feb. 29, 1944 |

#### OTHER REFERENCES

Page 364, Webster's New International Dictionary, second edition, 1939.